

## UNITED STATES PATENT OFFICE

LEON LILIENFELD, OF VIENNA, AUSTRIA

## VEGETABLE TEXTILE MATERIAL AND PROCESS FOR PRODUCING SAME

No Drawing. Application filed July 23, 1924, Serial No. 727,808, and in Austria April 4, 1924.

This invention relates to a new process for improving the quality of vegetable textile materials and particularly cotton, (or a fabric containing such a fibrous material).

5 According to the invention, very valuable properties are conferred upon woven or spun products of vegetable origin by treating them with a mono-halogen derivative of a fatty acid in the presence of an alkali.

10 The results of this process are: either a high degree of transparency and a silky lustre of a brilliancy hitherto unattained, or a more or less elastic or stiffening finish, or both lustre and finish.

15 Which of these effects is produced depends partly on the concentration and the proportions of the reagents, partly on the duration of the treatment, partly on the temperature, partly on the nature and previous treatment 20 of the fibrous material and partly on whether and at what stage in the process the material under treatment is stretched. When stretching is not employed substantially no silky lustre is produced, but instead the cotton fabric or yarn assumes a wool-like appearance 25 and feel respectively.

The process consists in treating a spun or woven fabric consisting of a vegetable fibrous material, particularly cotton, or a fabric containing such a fibrous material, with a mono-halogen-fatty acid or with a salt or derivative thereof (for example an ester) in the presence of an alkali. The spun or woven goods may be treated with alkali and halogen-fatty acid at the same time or in succession in either order.

As alkalies, there come into consideration in the first place the caustic alkalies. With alkali sulphides, however, results may be obtained, though these are less satisfactory.

40 All vegetable fibrous materials, such as linen, flax, hemp, ramie, jute, and particularly cotton, in the form of pure vegetable fabrics (for example pure cotton fabrics) or 45 of mixed fabrics or in the form of yarns in skeins or cops or of warps may be successfully treated according to the invention.

The textile material consisting of or containing vegetable fibre may be treated by the 50 present process either in crude state or after

a preliminary treatment (for example boiling, or heating under pressure with a solution of sodium carbonate or dilute caustic alkali or both), the textile material being previously moistened or not as desired, with or without previous extraction of the fatty matter, unbleached or bleached by means of an oxidizing or reducing bleaching agent, mercerized or not mercerized. It may also previously be prepared in known manner by means of a hydrolyzing or gelatinizing agent, for example, a strong mineral acid such as sulphuric acid of 49° to 60° Baumé gravity or phosphoric acid of 55° to 57° Baumé gravity, or 55 hydrochloric acid of 24° Baumé gravity, or 60 nitric acid of 43° to 46° Baumé gravity or more, or an ammoniacal solution of cupric oxide, or with a cold or hot solution of calcium thiocyanate or other thiocyanate. The preliminary treatment may consist in a combination of two or more of these methods. 70

In the present invention the working conditions may be varied within wide limits. It is therefore not to be limited to the details of the description hereinafter given of the 75 manner in which it is carried out.

The following methods of carrying out the process are given by way of example:—

The first consists in treating the spun or woven goods first with a solution of a caustic alkali and then with a monohalogen derivative of a fatty acid, such as monochloroacetic acid. The textile fibrous material may be treated with the alkali solution in various ways, for instance by immersing or soaking 80 the material in a small or large excess of alkali solution; or by immersing or soaking the material in the solution and removing the excess of the alkali solution by squeezing, centrifuging or the like; or by impregnating 85 in an impregnating mill or jigger or the like; or by padding by means of smooth or engraved rollers in a padding machine; or by coating by means of closely engraved rollers 90 in a Rouleaux machine in which case a suitable thickening medium is preferably used; or by spraying or by any other known 95 method.

As the alkali solution there may be used 100 for example caustic soda solution of 10-50

per cent strength. Caustic soda solutions of from 12 to 40 per cent strength have been found to be very suitable.

The quantity of the alkali solution which is incorporated in the spun or woven fabric or the quantity which is to be retained by the fabric may vary within very wide limits. Thus, for example, excellent results are obtained with an amount of twice or of ten times the weight of the textile material. As a rule an amount of from two to four times the weight of the textile material is found to be sufficient.

The temperature of the alkali solution may be selected from a wide range. According to the strength of the solution useful results are obtained at  $-10^{\circ}$  C. and from that up to  $+50^{\circ}$  C. In the case of alkali solutions which are not too weak satisfactory results are usually obtained at room temperature.

In order that the alkali solution may penetrate the fibres thoroughly and that the lustre may be improved the spun or woven goods may be allowed to pass between rollers during the treatment with the alkali solution or the material may be subjected to a high pressure in some other manner. If desired alcohol may be added to the alkali solution.

The textile material which has been treated with the alkali solution, immediately or after standing (ripening) for a short or long period (say 3 hours to 3 days) at or above room temperature is treated in the wet condition or after having been previously partially or completely dried, with a free monohalogen derivative of a fatty acid or with a salt or derivative (for example an ester) thereof. The monohalogen fatty acid or its salt, preferably alkali salt, may be brought into contact with the spun or woven goods which have been previously treated with alkali solution, in the form of a dilute or concentrated solution or of a supersaturated solution (for instance a pasty mass of crystals of an alkali metal salt) or of a suspension, or even in the solid form. As a solvent there may be used water or alcohol or a mixture of water and alcohol or any other solvent. In order to insure uniform distribution of the halogen fatty acid, or salt thereof, there may be added to the solution or suspension if desired a suitable binding or thickening agent, such as starch, dextrine, British gum, albumen or the like.

The monohalogen fatty acid, or the salt or derivative thereof may be added in various ways to the spun or woven goods which have been treated with the alkali solution. The goods may be soaked in the solution or suspension of the acid or of its salt in the cold or warmed to a temperature of for example  $50-100^{\circ}$  C. (in which case, if desired, any excess may be removed by squeezing or centrifuging); or they may be coated with it; or a solution or suspension of the halogen

fatty acid or salt or derivative thereof may be rolled into the textile material. Any other method, such as spraying, may however be used instead. In order to insure as uniform a distribution as possible of the acid or its salt throughout the textile material the latter may if desired be passed during the incorporation between one or more pairs of rollers, or otherwise subjected to pressure.

For the treatment with the monohalogen fatty acid there may be used any suitable device known in the cloth finishing or textile printing industry.

There is in practice no limit to the quantity of the halogen fatty acid or the salt, or derivative thereof, which may be used. As a rule, to which however the invention is not limited, it is sufficient to use not more than one or at the most two molecular proportions of monohalogen fatty acid for each molecule of caustic alkali. In most cases much smaller quantities, for instance 0.3 to 0.75 molecular proportion or even less, of the monohalogen fatty acid for each molecular proportion of caustic alkali is found to be sufficient.

The woven or spun goods which have been treated with the monohalogen fatty acid or with the salt or derivative thereof, either soon after the addition of the halogen fatty acid or after it has been in contact with it at room temperature or at a higher temperature (for example 50 to  $100^{\circ}$  C.) for a short or long time (for instance from half an hour to twenty-four hours) and after previously drying if desired, are then either directly washed or, advantageously, treated with a cold or warm solution of an inorganic or organic acid or of an acid salt, or of an ammonium salt, or of some other salt, or with a tannin solution, or with a formaldehyde solution or with any precipitating agent or mixture of precipitating agents known in the viscose industry or in the ammoniacal-copper-oxide-cellulose industry, and is then washed and dried. It may also be steamed before or after washing.

All the subsidiary operations usual in mercerization or proposed in connection therewith may also be employed in the present process, for instance lustering, pressure, mechanical beating and the like.

For the attainment of a high silk-like lustre, stretching of the textile fibrous material is essential. It may be stretched either during all the steps, that is, commencing with the impregnation with the alkali solution, up to the washing and drying process. Or it may be stretched only during the action of the alkali solution or of the halogen fatty acid; or the spun or woven goods may be stretched after the impregnation with alkali solution and kept stretched during the action of the halogen fatty acid and during the treatment with acid, salt, or the like and during the washing and final drying. Or they may be

stretched only after the action of the alkali solution and halogen fatty acid for the treatment with the acid or salt and the washing and optionally for the final drying. Or the 5 process may be conducted in such a way that the stretching is intermittent, the material being stretched for example, during the treatment with alkali solution, and with the acid or salt and the final washing, but not during 10 the action of the monohalogen fatty acid.

The second method of carrying out the process consists in reversing the order of the operations of the first method, that is to say, the textile fibrous material is first brought 15 into contact with the monohalogen-fatty acid or its salt or derivative and then introduced into the solution of alkali, or impregnated, coated or sprinkled or sprayed therewith. As 20 the halogen fatty acids exert no action on the fibrous material in the absence of alkali, the treatment with alkali solution may follow at leisure the treatment with the halogen fatty acid. After the material has been brought 25 into contact with the alkali solution the halogen fatty acid must be allowed to react for some time, and the action may proceed at or above room temperature. As regards 30 the other working conditions, such as the relative proportions of the reagents, temperature, duration of the reaction, stretching, 35 finishing of the goods and the like, the indications given in the description of the first method of carrying out the process are equally applicable.

The third method of carrying out the process consists in treating the textile fibrous material with a solution of the halogen fatty acid in alkali solution. This method, on account of the small power of resistance of the 40 monohalogen fatty acid to alkali hydroxide, is the least to be recommended. If it is desired to employ it, it is necessary to work either very quickly or at low temperatures (below 0° C. for example) or to use dilute 45 solutions of alkali.

By an appropriate selection of the conditions of working there may be obtained by the process silk-like effects which are far superior to those which may be obtained according to the usual mercerizing processes. In this case, if the quantities of the reagents are not excessively large and if the duration of the action of the monohalogen fatty acid is not carried too far, and if in the case of 55 a somewhat prolonged reaction the temperature employed is not unduly high, no stiffening, or substantially no stiffening of the fabric or yarn occurs. It acquires on the contrary, besides the silk-like lustre, a valuable 60 finish and elastic feel. The silk-like lustre may be materially enhanced by one or more repetitions of the process. Only by substantially increasing the quantities of reagents used; particularly in the case of the monohalogen fatty acid, and prolonging the dura-

tion of the action, especially at rather high temperatures, is a stiff finish obtained. Experience shows that when there are used alkali solutions of low or medium strength, caustic soda solutions of from 12 to 25 per 70 cent strength for example, even by the action of large quantities of monohalogen fatty acid, and even when the reaction is prolonged there is much less tendency towards the formation of a stiff finish than when strong solutions (30 to 50 per cent strength of caustic soda solution for instance) are used. 75

The dressing may further be increased by adding some cellulose, such as sulphite-cellulose or linters in a finely divided form, or 80 mercerized cellulose, or a cellulose hydrate, to the alkali solution (if desired, with the aid of a thickening agent) or to the solution, paste, or magma of the halogen fatty acid or salt thereof. 85

The process according to the invention is also suitable for obtaining pattern effects, for which purpose the following methods of procedure may be considered by way of example:—

(1) Before the treatment with the solution of an alkali a pattern is printed or stencilled on the woven fabric by means of a reserve paste which prevents absorption of the alkaline solution either mechanically or chemically. Appropriate reserve agents are, for example, albumen, gum, acids (such as acetic acid, citric acid, tartaric acid or an inorganic acid), alum, aluminium sulphate, ammonium sulphate or other salt. The fabric is then treated with an alkali solution and a monohalogen-fatty acid in the manner described in the first method of carrying out the process. This modification of the process gives rise to a lustrous pattern on a dull background, or vice versa. 100 105

(2) The alkali solution, mixed with an appropriate thickening medium (such as starch, denatured albumen, a cellulose hydrate soluble in alkali, alkyl or oxyalkyl derivative of cellulose soluble in alkali or in water, a cellulose ether of a mono-hydroxy carboxylic acid, or the like) is printed on the fabric in the form of any desired pattern, and the fabric is then treated with a halogen fatty acid in the manner already described. The effects obtained are similar to those in (1). 110 115

(3) The fabric, after being treated with alkali solution and, if desired, dried, is printed with a reserve which mechanically or chemically prevents the reaction between the alkali-cellulose and the halogen-fatty acid. As substances which are effective in this respect there may be used, for example, 120 an acid, albumen, kaolin, zinc white, or the like. A dyestuff or pigment may also be added to the reserve paste. After having been printed with the reserve material, the fabric is treated with the halogen fatty acid, 125 130

as described in the first method of procedure, treated with an acid or a salt, and dried. This method of working produces very lustrous effects on a less lustrous back-ground, 5 or vice versa.

(4) Pattern-effects may also be obtained by impregnating the fabric with a solution of an alkali, as described in the first form of the process, and then, after previously drying if desired, printing it with a monohalogen fatty acid or a salt thereof, dissolved or suspended in a suitable thickening medium (such as British gum, starch, or dextrine) with or without the addition of a dyestuff, 10 and then finishing the fabric as described in the first form of the process. Very lustrous effects are obtained on a less lustrous back-ground.

(5) A monohalogen fatty acid or a salt 20 thereof in the form of a solution or suspension is printed on the fabric with the aid of a thickening medium, after which the fabric is exposed with or without drying to the action of caustic alkali. The results obtained 25 are similar to those of (3) and (4).

The following examples illustrate the invention, the parts being by weight:—

I

(a) Bleached or unbleached cotton fabric 30 or yarn is treated with soda solution of 25-40 per cent strength at room temperature for a period of from 5 minutes to 12 hours and the excess of soda solution is removed by squeezing or centrifuging so that the fabric 35 retains about 2½ to 3½ times its weight, or any other desired quantity, of caustic soda solution. The material impregnated with the soda solution either immediately after the impregnation or after being left to itself for 40 from 3 to 72 hours, is then treated with sodium monochloracetate, prepared for example by dissolving 100 parts of monochloracetic acid in 100 parts of water or in a solution of British gum of 20 to 25 per cent 45 strength and adding to the solution about 90 parts of powdered sodium bicarbonate, in small portions whilst shaking or stirring. After addition of this quantity of bicarbonate and after the carbon-dioxide has escaped, a suspension of sodium chloracetate 50 crystals remains; this may be used as such, or after warming for a short time, for example to 50-60° C. during which it is converted into a solution. The yarn or fabric (carrying 55 the NaOH solution) may either be impregnated with the suspension or solution of sodium chloracetate or coated with it on one or on both sides, or the solution of the chloracetate may be rolled on or into the textile material. 60 The quantity of sodium chloracetate which is to be incorporated with the fabric or yarn impregnated with caustic soda solution is subject to variation between wide limits. For reasons of economy however it is desir- 65 able to use not more than from ½-1 part of

the weight of the cotton material, particularly as excellent effects may be obtained with these or even with smaller quantities. After the material has been in contact for a short time (for example, 10 minutes) or for a longer time (for example, 12 hours) with the sodium chloracetate it is introduced either into dilute sulphuric or acetic acid, for instance, of 10-20 per cent, or into a solution of ammonium chloride or ammonium sulphate of 20-30 per cent strength, or into any other precipitating bath customary in the viscose industry. It is allowed to remain in it for a short time (for instance 5 minutes) or for a longer time (for instance several hours), and is then washed and dried. The fixing agent may also be applied to the fabric by sprinkling, spraying, or the like. Or the cotton material is washed after it has been treated with alkali solution and sodium monochloracetate and then treated with the fixing agent, washed and dried. It may also be only washed and dried.

During the above operations the fabric or yarn should be stretched for at least a part of the time of treatment with the alkali solution or with the sodium chloracetate. If not too prolonged the material may be stretched throughout each operation. Otherwise it may be stretched only during the action of the soda solution or after impregnation with this solution, throughout the whole or a part of the duration of the action of the sodium chloracetate, and of the treatment with an acid or salt, if any. The textile fibrous material may also be washed in the stretched condition, this having a beneficial effect on the silk-like lustre.

According to this example there is obtained a high-grade silk-like lustre, and a pleasing, resilient finish; also, if the duration of the action of the alkali solution, or of the ripening, after the impregnation process, or of the action of the sodium monochloracetate is prolonged and the quantity of sodium monochloracetate is very large, a stiff finish is obtained.

(b) The procedure is as in Example I (a), with the difference that instead of the sodium chloracetate there is used an aqueous solution of free chloracetic acid of 50 per cent strength for impregnating or coating the material which has been impregnated with caustic soda solution.

(c) The procedure is as in Example I (a), with the difference that the sodium chloracetate is prepared as follows: 40 to 70 parts of chloracetic acid are dissolved in 160 to 130 parts of water or of a solution of British gum of 25-30 per cent strength and the solution is treated as in Example I (a), with about 36 to 63 parts of powdered sodium bicarbonate, whereby there is obtained a solution which is liquid at room tempera-

ture. The results obtained are somewhat similar to those obtained in the case of Example I (a).

- (d) The procedure is as in Examples I (a), I (b) or I (c), with the difference that the action of the sodium chloracetate or of the chloracetic acid as the case may be takes place while warm. For the purpose the fabric which has been impregnated with the caustic solution and brought into contact with the sodium chloracetate or chloracetic acid is maintained for a period of from 10 minutes to an hour at a temperature of 50° to 100° C., for example at 80° C. If the duration of the warming at 80° C. for example is prolonged for an hour or more there is obtained, besides a high-grade silky lustre, a stiff dressing, which may approximate to the stiffness of book-binder's linen.
- (e) The procedure is as in Examples I (a), I (b), I (c), or I (d), with the difference that instead of the caustic soda solution of 25-40 per cent strength there is used a caustic soda solution of 18-23 per cent strength, for example of 22.5 per cent strength. The finished products exhibit a very fine silk-like lustre.

- (f) The procedure is as in Examples I (a), I (c), I (d), or I (e), with the exception that the sodium monochloracetate or the like, preferably in the presence of British gum, is printed in the form of any desired pattern on the fabric which has been treated with caustic soda solution, and, if desired, dried before being printed.

## II

- (a) Bleached or unbleached cotton fabric or yarn is impregnated with a solution prepared as follows, with the addition, if desired, of a thickening medium such as British gum, as described in the foregoing examples:—100 parts of monochloracetic acid are dissolved in 400 to 900 parts of water and the solution is treated with about 90 parts of powdered sodium bicarbonate. The textile material impregnated with this solution is introduced if desired, after removing the excess by squeezing or centrifuging into a caustic soda solution, of 30-40 per cent strength left in contact with the solution for a period of from 10 minutes to two hours and then finished as described in Example I (a). The fabric is stretched during or after the treatment with the caustic soda solution. A silk-like lustre is obtained.

- (b) The procedure is as in Example II (a) with the difference that the material is dried before it is introduced into the caustic alkali solution.

## III

- The procedure is as in any of the Examples I (a) to I (e) with the difference that the sodium chloracetate is prepared in

the following manner: 90 parts of chloracetic acid are dissolved in 60 parts of water, and neutralized with about 80 parts of sodium bicarbonate which is added in small portions. As soon as the evolution of carbon-dioxide has ceased, 150 parts by weight of alcohol of 96 per cent strength are added whilst stirring, whereby a milky suspension is produced.

The silk effect produced is of a high grade, the finish has an elastic feel.

75

## IV

The procedure is as in any of the Examples I (a) to I (e), with the exception that instead of the aqueous caustic soda solution of 18 to 40 per cent strength there is used an alcoholic caustic soda solution of 18 per cent strength and having the following composition: 600 parts of aqueous caustic soda solution of 30 per cent strength, 85 400 parts of alcohol of 96 per cent strength.

The silk effect obtained is excellent.

## V

The procedure is exactly as in any of the preceding examples, with the modification that the material is first treated with a strong sulphuric acid prior to its treatment according to the process herein described. If a sulphuric acid of 49° to 50° Baumé gravity be used for this purpose, the treatment there-with may be allowed to proceed at room temperature for a period of from several seconds up to a few minutes and even longer. If a stronger sulphuric acid is used, for example, of 52° to 54° Baumé gravity, then the treatment must only occupy a few seconds, if the treatment is conducted at room temperature. If however the sulphuric acid be cooled down to 0° C. or below the treatment may continue for a longer period.

Mercerization of the fabric, for example, by means of a caustic soda solution of 10 per cent strength at a low temperature or with a strong caustic soda solution, for example, of 18 to 40 per cent strength, at room temperature, may precede the treatment with sulphuric acid.

## VI

The procedure is exactly as in any of the foregoing examples, with the difference that the fabric is previously mercerized according to any known mercerizing process.

Instead of the monochloracetic acid, there may be used with satisfactory results, a mono-halogen derivative of a homologue of acetic acid, such as  $\alpha$ -bromo-propionic acid,  $\alpha$ -bromo-butyric acid, or a halogen derivative of another organic acid, e. g. bromo-succinic acid.

The finished products may be calendered, schreined, or beetled or the like.

Examples for pattern effects by means of a reserve follow as a matter of course.

130

On treatment with a monohalogen derivative of a fatty acid in the presence of an alkali, the vegetable fibres are converted into a cellulose ether of an alkali salt of a mono-hydroxy carboxylic acid in which the cellulose has entered into the hydroxyl group of a monohydroxy carboxylic acid. In case of monochloracetic acid, cellulose ethers of alkali salts of glycolic acid are formed. Whether that conversion of the fibres takes place only on the surface of the fibres or in their deeper parts also, depends partly upon the concentration and amount of the alkali solution, partly on the quantity of the monohalogen-fatty acid used and partly on the temperature.

The cellulose ethers of alkali salts of mono-hydroxy carboxylic acids formed as indicated in the preceding paragraph will be converted into acid ethers by immersing the fabric in cold or warm solutions of organic acids, such as acetic acid, or by immersion in cold or warm dilute solutions of inorganic acids, such as dilute sulphuric acid, or by immersing the fabric in a solution of an acid salt or any precipitating agent or mixture of precipitating agents known in the viscose industry or in the ammoniacal-copper-oxide-cellulose industry.

On treating the finished fabric with a hot dilute mineral acid or a concentrated mineral acid at room temperature, a decomposition of the ethers takes place. This decomposition may be brought about, for example, by a hydro-halogen acid, such as hydrochloric acid, or by sulphuric acid. These mineral acids when used in the manner described cause the ethers of mono-hydroxy carboxylic acids or salts to liberate hydroxy-paraffin mono-carboxylic acids. Upon treating cellulose ether of glycolic acid with mineral acids in the manner above described glycolic acid is liberated.

The expression "textile fibrous material" in the specification and in the claims includes wherever the context permits, all vegetable fibrous materials, such as flax, linen, hemp, ramie-fibre, jute and particularly cotton and the like, in the form of pure vegetable fabrics 50 (for example pure cotton fabrics) or mixed fabrics or in the form of yarn in skeins, cops, or warps.

The expression "halogen derivative of fatty acid or monohalogen derivative of a fatty acid" includes wherever the context permits, the free monohalogen fatty acid or a salt, or a derivative thereof, such as an ester.

The expression "cellulose ether of a mono-hydroxy carboxylic acid" includes those cellulose compounds in which the cellulose has entered the hydroxyl group of a hydroxy-paraffin mono-carboxylic acid (possibly with the formation of a lactone or a lactide):

I claim:

1. As new products, vegetable textile fi-

brous materials which, without having been finished by means of a cellulose ether of a mono-hydroxy carboxylic acid supplied from outside, contain a cellulose ether of a mono-hydroxy carboxylic acid soluble in alkali, but 70 not in water.

2. As new products, vegetable textile fibrous materials which have a silk-like lustre and which, without having been finished by means of a cellulose ether of a mono-hydroxy 75 carboxylic acid supplied from outside, contain a cellulose ether of a mono-hydroxy carboxylic acid soluble in alkali but not in water.

3. As new products, vegetable textile fibrous materials, which, without having been 80 finished by means of a cellulose ether of glycolic acid supplied from outside, contain a cellulose ether of glycolic acid soluble in alkali but not in water.

4. As new products, vegetable textile fibrous materials which have a silk-like lustre and which, without having been finished by means of a cellulose ether of glycolic acid supplied from outside, contain a cellulose 85 ether of glycolic acid soluble in alkali but 90 not in water.

5. As new products, vegetable textile fibrous materials which, without having been finished by means of a cellulose ether of a mono-hydroxy carboxylic acid supplied from outside, split off a hydroxy-paraffin mono-carboxylic acid 95 on decomposition with a hydro-halogen acid.

6. As new products, vegetable textile fibrous materials which have a silk-like lustre and which, without having been finished by means of a cellulose ether of a mono-hydroxy carboxylic acid, supplied from outside, split off of hydroxy-paraffin mono-carboxylic acid 100 on decomposition with a hydro-halogen acid. 105

7. As new products, vegetable textile fibrous materials which, without having been finished by means of a cellulose ether of glycolic acid supplied from outside, split off glycolic acid 110 on decompositon with a hydro-halogen acid. 110

8. As new products, vegetable textile fibrous materials which have a silk-like lustre and which, without having been finished by means of a cellulose ether of glycolic acid 115 supplied from outside, split off glycolic acid on decomposition with a hydro-halogen acid. 115

9. The process of treating vegetable textile fibrous material which comprises subjecting said material to the action of a monohalogen derivative of a fatty acid in the presence of an alkali and preserving the textile character of said material throughout said action. 120

10. The process of treating cellulosic vegetable fibres which comprises subjecting said fibres to the action of a monohalogen derivative of a fatty acid in the presence of hydroxide of an alkali metal and regulating such action so that said fibres do not lose their 125 130

- identity as fibres but become converted at least in part into compounds of cellulose.
11. The process of treating cellulosic textile fibrous material which comprises subjecting said material to the action of a monohalogen derivative of a fatty acid in the presence of caustic alkali short of complete dissolution of the said cellulosic material, whereby said material becomes in part converted into a compound of cellulose, and thereafter converting the compound so formed into a water insoluble compound of cellulose.
12. The process of treating cellulosic textile fibrous material which has its fibres converted at least partially through their diameter into alkali cellulose which comprises subjecting the said so converted material to the action of a monohalogen fatty acid.
13. The process of treating cellulosic fibrous material which comprises converting the fibres of said material at least in part through their diameter into cellulose ether of a salt of mono-hydroxy carboxylic acid in which the cellulose has entered into the hydroxyl group of said salt, and thereafter converting said salt into the corresponding acid ether.
14. The process of treating cellulosic fibrous material which comprises subjecting said material to the action of a monohalogen acetic acid in the presence of an alkali only to such an extent that the fibres become finished with the cellulose derivative formed from said action.
15. The process of treating vegetable textile fibrous material which comprises subjecting said material to the action of monochloracetic acid in the presence of alkali and regulating the progress of said reaction so as not to destroy the initial character of said material as a textile.
16. The process of treating vegetable textile fibrous material which comprises subjecting said material to the action of a monohalogen derivative of a fatty acid and caustic alkali in two steps and preserving the textile character of said material throughout said action.
17. The process of treating vegetable textile fibrous material which comprises subjecting said material to the action of caustic alkali and thereafter to the action of a monohalogen derivative of a fatty acid and preserving the textile character of said material throughout the said actions.
18. The process of treating cellulosic fibrous material which comprises subjecting said material to the action of caustic alkali and thereafter to the action of a monohalogen acetic acid, and regulating said actions so that the fibres are not dissolved but merely finished with the cellulose derivative formed from said actions.
19. The process of treating cellulosic
- fibrous material which comprises subjecting said material to the action of a monohalogen fatty acid in the presence of alkali only to such an extent that the fibres become finished with a cellulose compound resulting from such action and thereafter converting said cellulose compound into a cellulose compound insoluble in water.
20. The process of treating vegetable textile fibrous material which comprises subjecting said material to the action of a solution containing caustic alkali, thereafter to the action of monochloracetic acid and regulating said actions to such an extent that the fibrous materials are not completely dissolved but retain their textile character and thereafter converting the cellulose compound formed by said action into a cellulose compound insoluble in water.
- In testimony whereof I affix my signature.
- LEON LILIENFELD.